

## UNITED STATES PATENT OFFICE.

DOUGLAS T. BEATTY, OF BIRMINGHAM, ALABAMA, ASSIGNOR TO SAND SPUN PATENTS CORPORATION, OF WILMINGTON, DELAWARE, A CORPORATION OF DELAWARE.

## METHOD OF CASTING.

No Drawing. Application filed May 15, 1925, Serial No. 30,609. Renewed June 25, 1926.

This invention is an improvement in methods of casting hollow bodies centrifugally, and more particularly in methods to prevent defacing of the inner surface of the casting through deposits of scruff and other impurities.

One of the problems involved in casting hollow metallic bodies, such as pipe, centrifugally is the tendency to the deposit of impurities, of specific gravity lower than that of the metal, which collect on the inner surface of the casting, usually near the ends.

Oxids to a greater or less degree in accordance with the nature of the metal, are continually forming on the surface while the molten metal is exposed to the atmosphere, and these together with other impurities, such as sand, slag and the like, because of their low specific gravity collect on the inner surface of the casting, in the form of scurf, scruff or scoria.

There is an especial tendency toward the formation of oxids during the rotation of the casting about its axis. As the fluid metal is carried up in the rotation, small particles are detached, and fall back into the molten metal at the bottom. In their fall through the mold atmosphere, which contains oxygen, a film of oxid forms on the surface, and since the fusing point of the metallic oxid is higher than that of the metal, the particles are not reincorporated in the molten bath into which they fall.

The impurities of low specific gravity, which under the combined influence of gravity and centrifugal force eventually attain the inner surface of the casting form a film, the fusing point of which like that of the film on the particles is higher than that of the metal, and the molten interior of the particles which is relatively pure metal, when it reaches the molten bath of similar metal, is separated therefrom by two films of a higher fusing point. Hence the relatively pure metal of the particle does not meet the relatively pure metal of the bath, to be re-united therewith in intimate union.

Such particles, or a relatively large proportion thereof, do not wholly penetrate the lining film of the casting, which film when cooled is scruff or scoria, but aggregate themselves with the same, greatly increasing the specific gravity of the film, so that it

more nearly approaches that of the metal in the casting.

Because of this approach to the same specific gravity of scruff and casting, there is not the clear separation between the two that is desirable. The union between the scruff layer and the casting wall is relatively intimate, the scruff bedding itself somewhat deeply into the casting wall, with a consequent weakening thereof, and pitting of the wall when the scruff is removed.

Many attempts have been made to remedy the conditions, which lead to the formation of scruff, and to the conditions above noted. It has been proposed to envelop the metal in a deoxidizing atmosphere, such for instance as carbon monoxide, hydrogen, steam or the like. This however is a process of some difficulty, requiring special machinery, and if entirely successful in the prevention of oxid formation, it does not in any way affect the other impurities which may be present, and which have a part in the formation of the scruff.

It has also been proposed to introduce at a suitable stage in the casting, an enameling material, in the endeavor to limit to some extent the formation of the scruff, and cover and conceal the imperfections it causes with a coating of enamel on the interior of the casting.

This process however, does not prevent the increase in specific gravity of scruff by the aggregation therewith of metallic iron, and the consequent blurring of the line of separation between the scruff and the casting wall. The coat of enamel also materially alters the appearance of the inner surface of the casting, so that it no longer presents the desirable natural iron color.

One of the primary objects of the present invention is the provision of a method of casting, wherein the impurities of the molten metal are converted into an extremely fluent slag with a very low melting point, which forms a coating on the surface of the molten metal, cooling into a superficial soluble facing on the inside of the casting.

Another object is the provision of a method, wherein the means for converting the impurities into slag is of such nature and so introduced that a non-oxidizing atmosphere is established and maintained in

the mold throughout the casting operation.

Another object is the provision of a method wherein by eliminating to a large degree the tendency toward the formation of oxids and the consequent aggregation of metallic iron with the scruff, the specific gravity of the scruff is maintained at a level such that there will be a distinct line of demarcation between the scruff and the metal, thus facilitating the removal of the scruff, and eliminating pitting.

Other objects will be in part obvious, and in part pointed out in the detail description, it being understood that many changes may be made in the materials used, in the proportions and in the time and order of their introduction, within the scope of the appended claims.

In the usual procedure of casting hollow bodies centrifugally, the molten metal in a desired state of fluidity is introduced into a refractory mold of any suitable character, such as sand, and the mold may be either inclined at the commencement of the introduction, or otherwise placed, as may be desired.

During the introduction, and for a time afterwards, the pipe is rotated at selected speeds, the rotation causing the metal to flow circumferentially of the mold, and to distribute itself evenly and uniformly over the mold surface, from end to end thereof. The impurities, such as oxids, sand, slag, and the like, are of lower specific gravity than the metal, and as a consequence they collect on the inner surface of the casting usually near the ends, cooling into stiff, heavy, viscous facing of scruff or scoria, more or less intimately attached to the metal of the casting. The coating is somewhat difficult to remove, and because the line of demarcation between the coating and the metal is not uniform, pitting and weakening of the casting wall may result.

I have discovered that by introducing any selected one or more of a number of materials of the character known as fluxes into the mold while the metal is still fluid, and preferably at some period of the pouring operation, a number of very desirable ends may be attained, among which may be mentioned the scavenging of impurities from the molten metal and the scavenging of oxidizing gases from the mold.

The fluxes have a very low fusing point, and immediately they strike the molten metal they fuse, spreading thereover, collecting impurities already present, such as slags, oxidized iron, sand and the like, fusing such impurities and forming with them a thin fluent slag, which blankets the surface of the metal, preventing the access of air thereto, and the consequent formation of metallic oxids.

The flux or fluxes also through fusion evolve an inactive gas, such as carbon dioxid, which drives out the gases already in the mold, and which contain oxygen, thus scavenging the mold, and establishing and maintaining an atmosphere which is at least inactive, so that no further oxidization of the surface metal will take place.

Because of the low specific gravity of the slag, it remains on the surface of the molten metal, picking up the impurities as they are moved under the influence of gravity and centrifugal force to the interior of the mold, and because of its low fusing point, it remains liquid until long after the metal is set, continuing to evolve inactive gases, and to function as scavenger for the metal and for the mold atmosphere.

There is a wide divergence in specific gravity between the slag produced by the flux and the metal, so that there is no tendency toward an intimate union between the two, and the line of demarcation is well defined, and substantially uniform, thus enabling the easy separation and removal of the slag, leaving a clean iron surface of the natural color.

The coating of slag is wholly superficial, with none embedded in the casting wall. When the casting is cooled, the coating is easily removed, adhering but loosely to the wall, and detached by jarring or scraping. The coating is in fact soluble in water, and may be removed by water treatment if desired.

The fluxing or slagging material may be introduced in any suitable manner, and at any stage while the metal is fluid. Obviously, however, the earlier it is introduced and the nearer to the ladle the point of introduction, the less opportunity there will be for the formation of oxids, and the longer time for the performance of the intended function.

Preferably the introduction of the said material is simultaneous with the introduction of the molten metal into the mold. When casting in an inclined mold, the flux may be delivered in a suitable stream onto the metal as it flows into the mold. When casting in molds otherwise arranged, the point and time of introduction will be governed by conditions, and the ends to be attained.

Any suitable fluxing compound may be used, such as sodium tetraborate (common borax), sodium chloride (table salt) or crude sodium carbonate (soda ash). In some respects, the last is preferable.

The quantity used depends to some extent upon the character of the metal, and the ends sought. With soda ash, the quantity for a 12 foot length of 4 to 6 inch pipe will vary from  $\frac{1}{2}$  to  $1\frac{1}{2}$  pounds. Usually about

1/2 pound is sufficient. Soda ash in pulverized form is preferably placed on the metal in the ladle just prior to casting. The soda ash fuses or melts down and becomes fluid 5 at a relatively low temperature, so that it is almost immediately converted to a fluid state, floating on top of the molten iron, and running into the mold with the iron, while retaining its surface position.

10 The gases given off during the slagging procedure, which is not entirely complete when the metal enters the mold, provide an inactive atmosphere in the mold. The slag floats on the inner face of the pipe, and 15 works its way toward the ends of the pipe or casting, just as the scruff has always done, and it may be easily removed after the cooling of the casting.

It will be evident from the description 20 that the flowing molten metal is surface coated with a fluxing or slagging material during charging of the mold. The slag formed collects to itself the scruff, foreign material such as sand, and the oxidized iron, 25 holding them in suspension on the surface of the iron. The formation is a true slag containing no metallic iron, and leaving beneath it a smooth surface when removed.

The desirable results attained by the use 30 of the fluxing or slagging material, introduced at the time, and in the manner described are manifold. Considered merely as a blanket of fusible material lying on the molten surface, the slag prevents access of 35 air to the metal, and the consequent formation of oxids. With the material used however, there is in addition an evolution of inactive gas, produced by the reaction of the fused sodium carbonate with such silica as 40 may be present, represented by the formula,



This reaction takes place in the ladle, and 45 in the mold, as rapidly as silicious material is available.

The stiff, heavy, viscous mass of scoria, sand and the like is converted into a thin, light, fluent slag in the reaction, which has a specific gravity about 1/3 that of the metallic 50 iron. Metal particles falling back from the top of the mold into the metal below are not oxidized in their fall, and pass readily through the thin slag blanket into the clean pool of metal, and are integrally incorporated therewith. After cooling, the slag 55 may be dissolved in water, and the entire deposit will be superficial, with none embedded in the metal. When entirely cooled, the slag is brittle like glass, and when removed exposes the natural clean face of the 60 metal.

The castings produced in accordance with 65 the method are of exceptional soundness, and homogeneity and free from all foreign materials. These desirable characteristics, are

due to the fact that the molten iron is in a condition of exceptional fluidity, enabling it to spread itself uniformly throughout the mold, and enabling it also to expel lighter materials, such slag, gas and the like, such 70 impurities passing freely through the fluent metal. The slag produced is also an exceptionally active scavenger, easily converting the foreign material into the fluid state.

In the practice of the improved method, 75 castings of greater tensile strength are obtained than by the usual methods, and with economy of operation. There is a saving of fuel, in that the desired temperatures are more easily obtained with the use of the 80 slagging material. That is the metal can be poured at a lower temperature than formerly, on account of the lack of resistance from scruff.

Because of the fact that the metal is purified in the practice of the method, iron with a relatively low carbon content may be used in the casting and perfect distribution obtained, which permits the making of castings 85 of greater tensile strength without sacrifice 90 of ability to resist bending stress, since the tensile strength of cast iron is controlled by the carbon content.

No claim is made in the present application to the product produced by the method, 95 the product being the subject matter of a separate application filed on June 10th, 1926, Serial No. 115,117.

I claim:

1. The step in the method of centrifugally casting hollow bodies, which consists in evolving inactive gas within the mold during the introduction of the molten metal, thereby to eject oxidizing gases which may be already present. 100

2. The step in the method of casting hollow bodies centrifugally, which consists in introducing with the molten metal a material forming when fused with silica a non-oxidizing 105 gas thereby to eject oxidizing gases which may be present. 110

3. The step in the method of casting hollow bodies centrifugally, which consists in introducing with the molten metal a fluxing or slagging material forming when fused with silica a non-oxidizing gas thereby to eject oxidizing gases which may be present. 115

4. The step in the method of casting hollow bodies centrifugally, which consists in introducing into the mold while the metal is still fluid a fluxing material capable of evolving a non-oxidizing gas during fusion with silica, and capable of forming with oxids and other impurities which may be present in the molten metal a slag. 120

5. The step in the method of casting hollow bodies centrifugally, which consists in introducing into the mold while the metal is fluid a material forming when fused with silica a non-oxidizing gas and combining with the 125

impurities of the metal to form a slag thereby to simultaneously scavenge the mold and the metal.

6. The step in the method of casting hollow bodies centrifugally, which consists in introducing a flux with the molten metal.

7. The step in the method of casting hollow bodies centrifugally, which consists in introducing into the mold a flux, while the metal is fluid.

8. The step in the method of centrifugally casting hollow bodies, which consists in floating a fluxing or slagging material on the flowing metal while the mold is being charged.

9. The step in the method of centrifugally casting hollow bodies, which consists in surface coating the flowing molten metal with a fluxing or slagging material.

10. The step in the method of centrifugally casting hollow bodies which consists, in slagging the impurities while the metal is flowing.

11. The method of centrifugally casting hollow bodies which consists in slagging the impurities while the metal is flowing with a material evolving a non-oxidizing gas during fusing with silica.

12. The step in the method of centrifugally casting hollow bodies, which consists in surface coating the flowing metal with a flux evolving a non-oxidizing gas during fusing with silica.

13. The step in the method of centrifugally casting hollow bodies, which consists in simultaneously scavenging the metal and the mold while the metal is flowing.

14. The method of preventing pitting in centrifugally cast hollow bodies, which comprises surface coating the molten metal during the charging of the mold with a flux to convert scuff forming impurities into slag, and removing the slag when the casting is cool.

15. The step in the method of centrifugally casting hollow metallic bodies in refractory molds, which consists in adding to the flowing metal a flux capable of forming with the impurities thereof a fluent slag to blanket the surface of the metal in the mold against oxidization by the air.

16. The step in the method of centrifugally casting hollow metallic bodies in refractory molds, which consists in adding to the flowing metal a flux capable of forming with the impurities thereof a fluent slag to blanket the surface of the metal in the mold against oxidization by the air, and capable of evolving when fused with silica an inactive gas to drive out the gases in the mold, thereby to establish and maintain a non-oxidizing atmosphere.

Signed at Birmingham in the county of Jefferson and State of Alabama, this 5th day of May, A. D. 1925.

DOUGLAS T. BEATTY.